# EUROPEAN PATENT APPLICATION

(11) **EP 4 394 072 A1**
(43) Date of publication of application: **03.07.2024**
(21) Application number: 22881305.1
(22) Date of filing: 11.10.2022
(51) Int. Cl.: C22C 38/02, C22C 38/04, C22C 38/06, C22C 38/60, C22C 38/14, C22C 38/00, B21C 23/08, C21D 9/52

(54) **SULFUR-ADDED GRAPHITE STEEL WIRE ROD, STEEL WIRE AND GRAPHITE STEEL, WHICH HAVE EXCELLENT CUTTING PERFORMANCE, AND MANUFACTURING METHODS THEREFOR**

(30) Priority: 12.10.2021 KR 20210135091
(71) Applicant: POSCO Co., Ltd, Pohang-si, Gyeongsangbuk-do 37859 (KR)
(72) Inventor: CHOI, Sangwoo, Pohang-si Gyeongsangbuk-do 37664 (KR)
(74) Representative: Nederlandsch Octrooibureau
(86) International application number: PCT/KR2022/015274
(87) International publication number: WO 2023/063678

(57) **Abstract**

The disclosure relates to a graphite steel wire rod, steel wire, graphite steel and manufacturing methods therefor to which sulfur is added and which have excellent cutting performance to that conventional free-cutting steel. Specifically, the disclosure relates to a graphite steel wire rod and steel wire, and manufacturing methods therefor, the rod and the wire comprising, by wt%, 0.60-0.90% of carbon(C), 2.0-2.5% of silicon(Si), 0.1-0.6% of manganese(Mn), 0.015% or less of phosphorus(P)(excluding 0), 0.031-0.3% of sulfur(S), 0.10-0.05% of aluminum(Al), 0.005-0.02% of titanium(Ti), 0.005-0.0020% of boron(B), 0.0030-0.0150% of nitrogen(N), and the balance of Fe and inevitable impurities. In addition, the present invention relates to graphite steel and a manufacturing method therefor, the steel comprising is same as above, having, as a microstructure, graphite grains distributed in a ferrite matrix, having a degree of graphitization of 90% or more, and containing 5% or less of MnS inclusions and pearlite in total.

## Description

### [Technical Field]

The disclosure relates to a graphite steel wire rod, steel wire and graphite steel having superior cutting performance and manufacturing methods thereof, and more particularly, to a sulfur-added graphite steel wire rod, steel wire and graphite steel having better cutting performance than common free-cutting steel and manufacturing methods thereof.

### [Background Art]

As a material for e.g., machine parts requiring machinability, free-cutting steel, to which machinability imparting elements such as Pb, Bi, and S are added, is commonly used. To improve machinability of steel materials, low melting point machinability imparting elements such as Pb and Bi are added to the steel to take advantage of the phenomenon of liquid metal embrittlement or a large amount of MnS is formed in the steel, and this free-cutting steel has superior machinability of the steel in terms of surface roughness, chip treatment, life of cutting tool during the cutting process.

However, Pb-added free-cutting steel that has the best machinability emits harmful substances such as toxic fumes while being cut, which is very harmful to the human body and is very unfavorable for recycling of the steel. Hence, to replace this, addition of S, Bi, Te, Sn, etc., is proposed, which is, however, known to have many problems in that production is difficult because cracking occurs easily while manufacturing the steel material or occurrence of cracks is caused during hot rolling.

As a free-cutting steel developed to solve the aforementioned problem, there is a graphite steel, and the graphite steel is a steel that contains fine graphite grains in a ferrite matrix or a ferrite-pearlite matrix, and the fine graphite grains act as crack sources to serve as chip breakers, thereby imparting good machinability.

However, despite this advantage of the graphite steel, the graphite steel has not yet commercialized. This is because when carbon is added to the steel, cementite, which is a metastable phase, is precipitated even though the graphite is a stable phase, so precipitation of the graphite without a separate long-term heat treatment for 10 or more hours is difficult, and in the long-term heat treatment process, decarburization occurs, causing adversely effects the final product performance.

In addition, even when graphite grains are precipitated through the graphitization heat treatment but when they are non-uniformly distributed in an irregular form, property distribution in cutting is irregular, resulting in very poor chip treatment or surface roughness, and further reducing the life of cutting tool, so it is hard to take advantage of the graphite steel. Accordingly, there is a need to provide a method of manufacturing a graphite free-cutting steel with superior machinability by using MnS based inclusions as well as graphite grains.

### [Disclosure]

### [Technical Problem]

The disclosure provides a sulfur-added graphite steel wire rod, steel wire, and graphite steel with superior machinability, and a manufacturing method thereof.

### [Technical Solution]

According to an embodiment of the disclosure, a graphite steel wire rod includes, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

According to another embodiment of the disclosure, a method of manufacturing a graphite steel wire rod includes manufacturing a billet including, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities; heating the billet; hot-rolling the heated billet to be manufactured into a wire rod; and cooling the wire rod.

According to another embodiment of the disclosure, a graphite steel wire includes, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

According to another embodiment of the disclosure, a graphite steel includes, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities, wherein as a microstructure, graphite grains are distributed in a ferrite matrix, a graphitization rate is at least 95%, and a total of 5% or less of MnS inclusions and pearlite are included.

According to another embodiment of the disclosure, a method of manufacturing a graphite steel includes manufacturing a wire rod including, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities; and performing graphitization heat treatment on the manufactured wire rod.

### [Advantageous Effects]

According to the disclosure, a graphite steel having superior machinability may replace the existing free-cutting steel and may be used as an eco-friendly free-cutting steel that replaces a harmful element such as Pb.

### Best Mode

According to an embodiment of the disclosure, a graphite steel wire rod includes, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

### Modes

A graphite steel wire rod, steel wire and graphite steel with superior machinability and a manufacturing method thereof according to the disclosure will now be described in detail.

### [Graphite steel wire rod]

According to an embodiment of the disclosure, a graphite steel wire rod includes, in percent by weight (wt%), 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

A unit of wt% will now be used unless otherwise mentioned. The term "include (or including)" or "comprise (or comprising)" is inclusive or open-ended and does not exclude additional, unrecited elements or method steps, unless otherwise mentioned.

### [Ranges of Ingredients]

### Carbon (C): 0.60 to 0.90wt%

Carbon is an essential element to form graphite grains. In a case that carbon content is less than 0.60wt%, the machinability enhancement effect is not enough and the distribution of the graphite grains is irregular even after completion of graphitization, and in a case that the content is in excess of 0.90wt%, it is likely that the graphite grains are formed coarsely and machinability, surface roughness in particular deteriorates due to an increase in aspect ratio. Accordingly, it is desirable that the carbon content has an upper limit of 0.90wt%.

### Silicon (Si): 2.0 to 2.5wt%

Silicon is actively added because it is a component required as a deoxidizer in manufacturing molten steel and a graphitization promoting element to precipitate the carbon as graphite by unstabilize cementite in steel. In the disclosure, to have this effect, it is desirable that the silicon content is at least 2.0wt%. Otherwise, when the content is excessive, not only the effect may be saturated but also it is likely that the hardness increases due to a solid solution strengthening effect, leading to acceleration of tool wear, brittlement is caused by an increase of nonmetallic inclusions and excessive decarburization is caused during hot rolling. Accordingly, it is desirable that the silicon content has an upper limit of 2.5wt%.

### Manganese (Mn): 0.1 to 0.6wt%

Manganese improves strength and impact properties of steel materials and contributes to machinability enhancement by combining with sulfur in steel and forming MnS inclusions. In the disclosure, to have this effect, it is desirable that manganese is contained in at least 0.1wt%. On the other hand, when the content is excessive, it may interfere with graphitization, delaying graphitization completion time and may increase the strength and hardness, thereby deteriorating machinability. Accordingly, it is desirable that the manganese content has an upper limit of 0.6wt%.

### Phosphorus (P): 0.015wt% or less (except 0)

Phosphorus is an impurity unavoidably contained. Although phosphorus helps machinability by weakening grain boundaries of steel, it increases hardness of ferrite through a significant solid solution strengthening effect, reduces toughness and delayed fracture resistance of the steel and promotes occurrence of surface defects, so it is desirable to maintain the content as low as possible. It is advantageous to control the phosphorus content to be 0wt% in theory, but the phosphorus is inevitably contained in a manufacturing process. Hence, it is important to manage the upper limit, and in the disclosure, the upper limit is kept to 0.015wt%.

### sulfur (S): 0.031 to 0.3wt%

Sulfur has a machinability enhancement effect with creation of MnS, but when contained in excess, mechanical anisotropy appears due to MnS elongated by rolling. In the disclosure, production of MnS was induced by adding sulfur within a range that may contribute to improving machinability without causing the mechanical anisotropy. Specifically, when sulfur is included in the range of 0.031 to 0.3wt%, MnS is generated and machinability is improved, and 100% of cutting performance appears as compared to lead free-cutting steel. However, when the content of sulfur is controlled to less than 0.03 1wt%, it leads to a failure of making a fraction of MnS inclusions enough to improve the cutting performance. Furthermore, when it exceeds 0.3wt%, anisotropy of the material increases, causing breakage during the cutting process, which incurs a risk during the processing.

### Aluminum (Al): 0.01 to 0.05wt%

Aluminum is a second element that promotes graphitization after silicon. This is because aluminum makes cementite unstable when it exists as solid solution Al, so it needs to exist as the solid solution Al. In the disclosure, to have this effect, it is desirable to contain at least 0.01wt%. On the other hand, when the content is excessive, not only is the effect saturated, but it may also cause nozzle clogging during continuous casting and AIN is formed at the austenite grain boundaries, so graphite with the AlN as the nucleus is distributed non-uniformly at the grain boundaries. Accordingly, it is desirable that the aluminum content has an upper limit of 0.05wt%.

### Titanium (Ti): 0.0051 to 0.02wt%

Titanium is combined with nitrogen together with boron, aluminum, etc., to produce nitrides such as TiN, BN, AIN, etc., and the nitrides act as nuclei for graphite formation during isothermal heat treatment. However, BN, AIN, etc., have a low formation temperature and are precipitated irregularly at the grain boundaries after austenite is formed, whereas TiN has a higher formation temperature than AIN or BN and is crystallized before austenite formation is completed, so it is uniformly distributed at the austenite grain boundaries and within the grains. Therefore, the graphite grains produced using TiN as the nucleation site are also distributed finely and uniformly. To have this effect, it is desirabe to contain at least 0.0051wt%, but when the content is added in excess of 0.02%, they become coarse carbonitrides that consume carbon required to form graphite, thereby inhibiting graphitization. Accordingly, it is desirable that the titanium content has an upper limit of 0.02wt%.

### Nitrogen (N): 0.0030 to 0.0150wt%

Nitrogen combines with titanium, boron and aluminum to produce TiN, BN, AIN, etc., and the nitrides such as BN, AlN, etc., in particular are mostly formed at austenite grain boundaries. During graphitization heat treatment, graphite is formed with these nitrides as nuclei, which may cause non-uniform distribution of graphite, so an appropriate amount of addition is necessary. When an amount of nitrogen added is excessive, it may not combine with nitride forming elements, and when it exists in steel as solid solution nitrogen, it adversely acts to delay graphitization by increasing strength and stabilizing cementite. Accordingly, in the disclosure, the nitrogen content was limited to 0.0030wt% as a lower limit and 0.0150wt% as an upper limit in order to consume them to form nitrides that act as graphite nucleation sites and not to leave them as solid solution nitrogen.

### Boron (B): 0.0005 to 0.0020%

It is actively added because it combines with N to form BN, which acts as a nucleus for crystallization of graphite and promotes graphitization, but the effect is small at less than 0.0005wt% and when it is added in excess of 0.0020wt%, excessive BN is formed at austenite grain boundaries, not only causing non-uniform distribution of graphite grains after graphitization heat treatment but also weakening the grain boundaries and then significantly reducing hot rolling properties, so it is desirable to contain boron in a range of 0.0005 to 0.0020wt%.

In the disclosure, the remaining ingredients are iron (Fe) and unavoidable impurities. This may not be excluded because unintended impurities may be inevitably mixed from raw materials or surroundings in the normal steel manufacturing process. These impurities may be known to anyone skilled in the ordinary steel manufacturing process, so not all of them are specifically mentioned in this specification.

Furthermore, in an embodiment of the disclosure, a wire rod for graphitization heat treatment may have an area fraction of pearlite of at least 95%. In the disclosure, graphite grains are produced by decomposition of pearlite, so when the area fraction of pearlite is low, the fraction of graphite grains is also bound to be low, showing non-uniform distribution, which is undesirable. As it is advantageous to have a high area fraction of pearlite to secure uniform and fine graphite grains, the upper limit is not particularly limited.

### [Method of manufacturing wire rod]

In an embodiment of the disclosure, a method of manufacturing a graphite steel wire rod includes manufacturing a billet including, in percent by weight (wt%), 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities;
heating the billet;
hot-rolling the heated billet to be manufactured into a wire rod; and
cooling the wire rod.

### Wire rod heating process

In an embodiment of the disclosure, the heating may include performing heat treatment by maintaining at a range of 1050 ± 100 °C for at least 60 minutes.

Before wire rod rolling, the billet is maintained at a range of 1050 ± 100 °C for at least 60 minutes. It is disadvantageous at a low heating temperature because the rolling load may increase at less than 950 °C of heating temperature of the billet, which reduces rolling productivity. When the heating temperature exceeds 1150 °C, it not only increases the expense but also accelerates decarburization, making the decarburized layer thickened, which undesirably remains even in the final product. The reason for setting the heating holding time to at least 60 minutes is that it is difficult to secure uniform temperature distribution in and outside the billet for wire rod rolling during less than 60 minutes.

### Wire rod rolling process

In an embodiment of the disclosure, the hot-rolling the billet to be manufactured into a wire rod may include hot-rolling at a temperature range of 900 to 1150 °C.

The reason for setting the wire rod rolling temperature into a range of 900~1150°C is that surface blemishes may easily occur during hot rolling or rolling may be hard because the rolling load increases at less than 900 °C, and that austenite grain size (AGS) becomes coarse at higher than 1150°C, increasing graphitization heat treatment hours after wire rod rolling.

### Cooling process

In an embodiment of the disclosure, the cooling may include cooling down to 500 °C at 0.1~10.0°C/s.

Furthermore, an embodiment of the disclosure may further include air cooling after the cooling.

At a cooling rate that exceeds 10.0 °C, it is undesirable because a hard phase such as martensite is generated and wire breakage may occur during cold drawing, which is a process following wire rod rolling, and at a cooling rate of less than 0.1°C, it is undesirable because a proeutectoid phase is excessively generated, reducing the pearlite fraction or coarsening the grain size so that the graphite grains produced after the graphitization heat treatment may have a non-uniform distribution.

### [Graphite steel wire]

In an embodiment of the disclosure, a graphite steel wire includes, in percent by weight (wt%), 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

### [Graphite steel]

In an embodiment of the disclosure, a graphite steel includes, in percent by weight (wt%), 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities, wherein as a microstructure, graphite grains are distributed in a ferrite matrix, a graphitization rate is at least 95%, and a total of 5% or less of MnS inclusions and pearlite are included.

In the meantime, the graphitization rate refers to a ratio of the carbon content that exists in the form of graphite to the carbon content added to the steel and is defined by the following [relational equation 1], and at least 95% of graphitization means that most of the added carbon was used to form graphite (the amount of the solid solution carbon in ferrite and solid solution carbon in fine carbides is very tiny, so it is ignored), meaning that there is no undissolved pearlite, that is, it has a microstructure in which graphite grains are distributed in the ferrite matrix. Graphitization rate (%) = (1 - carbon content in undissolved pearlite / carbon content in steel) × 100

### (Graphitization rate is 100% when there is no undissolved pearlite)

### [Method of manufacturing graphite steel]

In an embodiment of the disclosure, a method of manufacturing a graphite steel includes manufacturing a wire rod including, in percent by weight (wt%), 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities; and
performing graphitization heat treatment on the manufactured wire rod.

In an embodiment of the disclosure, the performing of the graphitization heat treatment may include performing heat treatment at a range of 700 to 800 °C for at least 5 hours.

When the heat treatment is maintained at the range of 700 to 800 °C for at least 5 hours, the graphitization rate may reach at least 95%. On the other hand, at less than 700 °C, the graphitization heat treatment time increases and exceeds at least 10 hours, and at higher than 800 °C, not only does the graphitization time increases, but also austenite is generated due to reverse transformation of pearlite and pearlite may form again during cooling, both cases of which are not desirable.

### Embodiments of the disclosure will now be described in more detail.

The following embodiments are provided to deliver the idea of the disclosure to those of ordinary skill in the art, but the disclosure is not limited to the embodiments and may be implemented in other forms.

### (Embodiments)

A billet containing ingredients in table 1 below was maintained for 90 minutes under a heating temperature condition and subjected to high-speed wire rod rolling to be manufactured into a wire rod having a diameter of 19 mm. Wire rod cooling rate, area fraction of wire rod pearlite and graphitization heat treatment time and graphitization fraction for this case are shown in table 1 below.

In tables 1 and 2, embodiments 1 to 11 correspond to graphite steel wire rods that satisfy an alloy composition range and manufacturing conditions of the disclosure, and comparative examples 1 to 7 correspond to wire rods that do not satisfy the alloy composition range and/or manufacturing conditions of the disclosure.

**[Table 1]**

| | C | Si | Mn | S | Ti | B | P | Al | N | Cutting performa nce (%) |
|---|---|---|---|---|---|---|---|---|---|---|
| Embodime nt 1 | 0.65 | 2.1 | 0.25 | 0.14 | 0.01 5 | 0.00 06 | 0.005 | 0.015 | 0.005 | 100 |
| Embodime nt 2 | 0.87 | 2.15 | 0.36 | 0.24 | 0.01 7 | 0.00 15 | 0.008 | 0.023 | 0.008 | 100 |
| Embodime nt 3 | 0.72 | 2.35 | 0.47 | 0.03 5 | 0.00 7 | 0.00 08 | 0.006 | 0.043 | 0.010 | 100 |
| Embodiment 4 | 0.68 | 2.18 | 0.16 | 0.26 | 0.009 | 0.0009 | 0.009 | 0.035 | 0.009 | 100 |
| Embodime nt 5 | 0.82 | 2.25 | 0.55 | 0.05 | 0.01 2 | 0.00 12 | 0.012 | 0.040 | 0.014 | 100 |
| Embodime nt 6 | 0.62 | 2.48 | 0.50 | 0.09 | 0.00 6 | 0.00 18 | 0.014 | 0.042 | 0.012 | 100 |
| Embodime nt 7 | 0.73 | 2.42 | 0.2 | 0.16 | 0.01 1 | 0.00 07 | 0.009 | 0.034 | 0.006 | 100 |
| Embodime nt 8 | 0.78 | 2.32 | 0.32 | 0.19 | 0.01 6 | 0.00 17 | 0.008 | 0.019 | 0.008 | 100 |
| Embodime nt 9 | 0.85 | 2.15 | 0.48 | 0.27 | 0.00 9 | 0.00 11 | 0.004 | 0.027 | 0.013 | 100 |
| Embodime nt 10 | 0.75 | 2.26 | 0.14 | 0.21 | 0.01 8 | 0.00 1 | 0.010 | 0.030 | 0.007 | 100 |
| Embodime nt 11 | 0.73 | 2.46 | 0.41 | 0.15 | 0.00 8 | 0.00 15 | 0.012 | 0.020 | 0.008 | 100 |
| Comparati ve example 1 | 0.63 | 2.0 | 0.23 | 0.00 5 | 0.01 6 | 0.00 0 | 0.017 | 0.005 | 0.001 | 88 |
| Comparati ve example 2 | 0.68 | 2.2 | 0.35 | 0.00 3 | 0.02 | 0.00 02 | 0.020 | 0.006 | 0.002 | 95 |
| Comparati ve example 3 | 0.73 | 2.25 | 0.45 | 0.00 6 | 0.00 9 | 0.00 04 | 0.025 | 0.075 | 0.018 | 89 |
| Comparati ve example 4 | 0.95 | 2.15 | 0.3 | 0.00 7 | 0.01 8 | 0.00 25 | 0.023 | 0.060 | 0.020 | 92 |
| Comparati ve example 5 | 0.55 | 2.6 | 0.56 | 0.4 | 0.02 5 | 0.00 25 | 0.019 | 0.003 | 0.025 | 91 |
| Comparati ve example 6 | 0.8 | 2.75 | 0.9 | 0.45 | 0.03 | 0.00 24 | 0.018 | 0.065 | 0.021 | 93 |
| Comparati ve example 7 | 0.75 | 2.8 | 0.8 | 0.35 | 0.00 2 | 0.00 3 | 0.020 | 0.06 | 0.022 | 90 |

The cutting performance has a numerical value based on cutting performance of lead free-cutting steel (100% refers to an equivalent level).

**[Table 2]**

| section | wire rod | | | graphitization | |
|---|---|---|---|---|---|
| | Cooling start temperature (°C) | cooling rate (°C/s) | Area fraction of pearlite (%) | Holding time (hr) | Graphitizatio n fraction (%) |
| Embodi ment 1 | 880 | 0.5 | 95.1 | 6.5 | 99 |
| Embodi ment 2 | 865 | 7.5 | 96.5 | 8.1 | 99 |
| Embodi ment 3 | 815 | 1.5 | 95.1 | 7.5 | 100 |
| Embodi ment 4 | 795 | 3.2 | 96.0 | 5.5 | 100 |
| Embodi ment 5 | 865 | 5.0 | 97.5 | 9.4 | 100 |
| Embodi ment 6 | 850 | 2.0 | 95.5 | 5.6 | 99.5 |
| Embodi ment 7 | 795 | 9.0 | 96.5 | 6.4 | 100 |
| Embodi ment 8 | 755 | 4.5 | 96.0 | 7.2 | 98.5 |
| Embodi ment 9 | 890 | 6.0 | 96.5 | 8.5 | 100 |
| Compara tive example 1 | 915 | 0.05 | 93.0 | 1.5 | 75 |
| Compara tive example 2 | 865 | 12.0 | 93.5 | 2.5 | 85 |
| Compara tive example 3 | 815 | 11.5 | 94.2 | 3.0 | 86 |
| Compara tive example 4 | 740 | 0.07 | 93.2 | 2.5 | 85 |
| Compara tive example 5 | 880 | 15.5 | 93.5 | 3.4 | 86 |
| Compara tive example 6 | 830 | 14.0 | 94.1 | 4.2 | 84 |

The structure of (100% - graphitized fraction) consists of MnS inclusions and pearlite, and the graphitized structure consists of ferrite + graphite grains. It can be seen that the area fraction of pearlite and the graphitization fraction are attained under wire rod and graphitization manufacturing conditions as shown in table 2 above.

The embodiments and the comparative examples will now be evaluated with reference to tables 1 and 2.

Embodiments 1 to 11 satisfy the alloy composition range and manufacturing conditions of the disclosure, so that the area fraction of pearlite in the graphite steel wire rod is at least 95%, the graphitization rate is at least 98.5%, and the cutting performance is 100% as compared to lead free-cutting steel.

On the other hand, the cutting performance of the graphite steel of comparative example 1, in which the sulfur content was only 0.005wt% and no boron is substantially contained, was only 88% as compared to the lead free-cutting steel, and according to the method of manufacturing a wire rod of comparative example 1, a wire rod cooled at a cooling rate of 0.05 °C/s and including 93% of area fraction of pearlite was obtained and subjected to heat treatment for 1.5 hours, so that the graphitization fraction was only 75%.

The cutting performance of the graphite steel of comparative example 2, in which the sulfur content was only 0.003wt% and the boron content was only 0.0002wt%, was only 95% as compared to the lead free-cutting steel, and according to the method of manufacturing a wire rod of comparative example 2, a wire rod cooled at a cooling rate of 12.0 °C/s and including 93.5% of area fraction of pearlite was obtained and subjected to heat treatment for 2.5 hours, so that the graphitization fraction was only 85%.

The cutting performance of the graphite steel of comparative example 3, in which the sulfur content was only 0.006wt% and the boron content was only 0.0004wt%, was only 89% as compared to the lead free-cutting steel, and according to the method of manufacturing a wire rod of comparative example 3, a wire rod cooled at a cooling rate of 11.5 °C/s and including 94.2% of area fraction of pearlite was obtained and subjected to heat treatment for 3.0 hours, so that the graphitization fraction was only 86%.

The cutting performance of the graphite steel of comparative example 4, in which the carbon content was 0.95wt%, the sulfur content was 0.007wt% and the boron content was 0.0025wt%, was only 92% as compared to the lead free-cutting steel, and according to the method of manufacturing a wire rod of comparative example 4, a wire rod cooled at a cooling rate of 0.07 °C/s and including 93.2% of area fraction of pearlite was obtained and subjected to heat treatment for 2.5 hours, so that the graphitization fraction was only 85%.

The cutting performance of the graphite steel of comparative example 5, in which the carbon content was 0.55wt%, the silicon content was 2.6wt%, the sulfur content was 0.4wt%, the titanium content was 0.025wt% and the boron content was 0.0025wt%, was only 91% as compared to the lead free-cutting steel, and according to the method of manufacturing a wire rod of comparative example 5, a wire rod cooled at a cooling rate of 15.5 °C/s and including 93.5% of area fraction of pearlite was obtained and subjected to heat treatment for 3.4 hours, so that the graphite fraction was only 86%.

The cutting performance of the graphite steel of comparative example 6, in which the silicon content was 2.75wt%, the manganese content was 0.9wt%, the sulfur content was 0.45wt%, the titanium content was 0.03wt% and the boron content was 0.0024wt%, was only 93% as compared to the lead free-cutting steel, and according to the method of manufacturing a wire rod of comparative example 6, a wire rod cooled at a cooling rate of 14.0 °C/s and including 94.1% of area fraction of pearlite was obtained and subjected to heat treatment for 4.2 hours, so that the graphite fraction was only 84%.

Furthermore, the graphite steel of comparative example 7, which contained 2.8wt% of silicon, 0.8wt% of manganese, 0.35wt% of sulfur, 0.002wt% of titanium, and 0.003wt% of boron, was only 90% as compared to the lead free-cutting steel.

From the evaluation of the aforementioned embodiments and comparative examples, it can be seen that all the properties of the graphite steel wire rod and graphite steel in the disclosure may be satisfied only when the alloy composition range and manufacturing conditions in the disclosure are satisfied.

### [Industrial Applicability]

According to the disclosure, a graphite steel having superior machinability may replace the existing free-cutting steel and may be used as an eco-friendly free-cutting steel that replaces a harmful element such as Pb, so the industrial applicability is acknowledged.

## Claims

1. A graphite steel wire rod having superior cutting performance, the graphite steel wire rod comprising:
in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

2. The graphite steel wire rod of claim 1, wherein an area fraction of pearlite is at least 95%.

3. A method of manufacturing a graphite steel wire rod with superior cutting performance, the method comprising:
manufacturing a billet including, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities; and
heating the billet;
hot-rolling the heated billet to be manufactured into a wire rod; and
cooling the wire rod.

4. The method of claim 3, wherein the heating comprises performing heat treatment by maintaining at a range of 1050±100 °C for at least 60 minutes.

5. The method of claim 3, wherein the hot-rolling for manufacturing the wire rod comprises hot-rolling at a temperature range of 900 to 1150 °C.

6. The method of claim 3, wherein the cooling comprises cooling down to 500 °C at a cooling rate of 0.1 to 10.0 °C/s.

7. The method of claim 3, further comprising: air-cooling after the cooling.

8. A graphite steel wire having superior cutting performance, the graphite steel wire comprising:
in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities.

9. A graphite steel with superior cutting performance, the graphite steel comprising:
in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities,
wherein as a microstructure, graphite grains are distributed in a ferrite matrix, a graphitization rate is at least 95%, and a total of 5% or less of MnS inclusions and pearlite are included.

10. A method of manufacturing a graphite steel having superior cutting performance, the method comprising:
manufacturing a wire rod including, in percent by weight, 0.60 to 0.90% of carbon (C), 2.0 to 2.5% of silicon (Si), 0.1 to 0.6% of manganese (Mn), 0.015% or less (except 0) of phosphorus (P), 0.031 to 0.3% of sulfur (S), 0.01 to 0.05% of aluminum (Al), 0.005 to 0.02% of titanium (Ti), 0.0005 to 0.0020% of boron (B), 0.0030 to 0.0150% of nitrogen (N) and the remainder having Fe and unavoidable impurities; and
performing graphitization heat treatment on the manufactured wire rod.

11. The method of claim 10, wherein the performing graphitization heat treatment comprises performing heat treatment at a temperature range of 700 to 800 °C for at least 5 hours.
